

# United States Patent Office.

GRANVIL RICH, OF SMITHVILLE, MISSOURI.

*Letters Patent No. 77,828, dated April 28, 1868.*

## IMPROVED COMPOUND FOR TEMPERING CAST STEEL.

The Schedule referred to in these Letters Patent and making part of the same.

### TO ALL WHOM IT MAY CONCERN:

Be it known that I, GRANVIL RICH, of Smithville, in the county of Clay, and State of Missouri, have invented a new and useful Compound for Tempering Cast Steel; and I do hereby declare that the following is a full, clear, and exact description thereof.

The ingredients and proportions are as follows:

I take three and one-half pounds tallow, one pound beeswax, one and one-half pint sweet oil, one and one-half ounce sal-ammoniac, pulverized, one and one-half ounce sweet spirits of nitre, and one ounce cream of tartar.

I melt the tallow and beeswax together, and then add the oil, next the tartar, then the sal-ammoniac, and lastly the nitre. I pour into the compound slowly, stirring them well while pouring; and thus the compound is completed and ready for use.

To use the above-described compound, I heat the steel or tools to be hardened to a regular or common heat used for such purposes, and harden them by immersing them in the compound while in a melted state. I then draw the temper, after rubbing or cleaning the steel or tools bright, as follows, viz:

For mill-picks and engravers' tools, I draw to a light gold color.

For plane-bits, large, heavy broad-axes, and turners' chisels, a straw color.

For adzes, large hand-axes, large taps and dies, firmer-chisels and gouges, butchers' cleavers, and bits for braces, a copper color.

For drawing-knives, socket-chisels, tools for turning iron and steel, drills for drilling iron, stone-drills, points, and chisels, a copper color tinted with blue.

For a chopping-axe or pole-axe, take all the copper from the blue tint.

For springs, I heat the spring to a cherry red, and cool it in the compound, and then hold it over the fire until the same is burned off, and then lay it down to cool.

I carefully keep all of the above-named articles from water while in a hot state.

Having thus described my invention, and the manner of using it, I claim, and desire to secure by Letters Patent—

1. The compound, as described; and for the purposes specified.
2. The process of tempering steel by the use of said compound, as described.

GRANVIL RICH.

Witnesses:

T. C. THEAKER,  
ERASTUS SMITH.